

## [54] ZINC OXIDATION PROCESS

[75] Inventors: Nicolo Gugliemi; Settimo Vittone; Gianfranco Rolando, all of Turin, Italy

[73] Assignee: Ing. C. Olivetti & S.p.A., Torino, Italy

[22] Filed: June 8, 1972

[21] Appl. No.: 260,796

## [30] Foreign Application Priority Data

June 9, 1971 Italy ..... 68985/71

[52] U.S. Cl. ..... 204/56 R, 204/39

[51] Int. Cl. ..... C23b 9/00, C23b 5/00

[58] Field of Search ..... 204/39, 56 R, 14 N

## [56] References Cited

## UNITED STATES PATENTS

2,666,023 1/1954 Schaaber ..... 204/39

3,330,744 7/1967 Wright ..... 204/56 R

Primary Examiner—T. M. Tufariello  
Attorney, Agent, or Firm—I. J. Schaefer

## [57] ABSTRACT

The surface oxidation process of the zinc or of a zinc coating consists of immersion of the zinc in an electrolytic cell, where a direct current of selected magnitude is driven and where the electrolytic bath consists essentially of a solution in an alkali metal nitrate melted mixture either of an hexavalent oxide of the type  $XO_3$  or of a salt of the type  $Y_2XO_4$  or of a salt of the type  $Y_2Cr_2O_7$ , where X represents an element selected in the group of chromium molybdenum and tungsten and Y an element selected between sodium and potassium. When solution of hexavalent chrome  $CrH_3$  in a mixture of melted alkali metal nitrates is used as bath, the oxidizing process can be carried out without current in the cell, by mere immersion of the zinc.

10 Claims, 1 Drawing Figure





Corrosion phase {

- red oxidation
- white oxidation
- discolouration phase

## ZINC OXIDATION PROCESS

## BACKGROUND OF THE INVENTION

The present invention relates to a method of oxidizing the surface of an article having at least a surface layer of zinc.

One of the most widespread surface treatments for improving the corrosion resistance of steel is that of galvanizing by plating with zinc. It has been found that a longer life for the protective zinc layer may be attained by the anodic oxidation or the passivation of the layer.

Typical conventional methods for anodic oxidation of the zinc involve the use of electrolytes such as a relatively diluted aqueous solution of ammonia, sulfuric acid, chromic acid, and ammonium fluoride. The layers attainable by these methods show adequate corrosion resistance, but they lack good mechanical characteristics and require high formation voltages (from 90 to 200 V).

Baths of melted nitrate mixture have been used successfully for the anodic oxidation of aluminum and of the valve-metals (namely, the metals showing a high surface resistivity in the anodic direction and a low surface resistivity in the cathodic direction when used as electrodes in an electrolytic cell, such as aluminum, tantalum, zirconium, niobium). However, such baths cannot be used for zinc inasmuch as the anodic current produces the dissolution of the zinc itself.

Passivation is normally executed by a chemical process involving immersing the zinc in an aqueous solution having a chromate basis and produces oxide and chromate layers on the zinc surface having a rather complex structure. Such processing imparts a certain atmospheric corrosion resistance to the layer, but the resulting passivated layers are very thin and have little resistance to abrasion.

## SUMMARY OF THE INVENTION

The disadvantages of the prior methods are obviated by the method of the present invention which provides a new method for the anodic oxidation of a zinc surface in which the electrolytic bath comprises a mixture of melted alkali metal nitrates and/or alkaline earth metal nitrates with the addition of a selected quantity of an oxidizing additive.

According to another aspect of the present invention a zinc surface may be passivated by immersion in a bath comprising a solution of hexavalent chrome oxide  $\text{CrO}_3$  in a mixture of melted alkali metal nitrates and alkaline earth metal nitrates.

## BRIEF DESCRIPTION OF THE DRAWING

The Drawing displays the results of corrosion resistance tests of zinc plated sheet metals processed by the method of the invention.

## DETAILED DESCRIPTION

In the process according to the invention, the object whose zinc surface is to be oxidized is degreased and immersed in an electrolytic cell wherein the electrolyte comprises a solution of an oxidizing substance in a mixture of melted salts. The salts may be alkali metal nitrates and/or alkaline earth metal nitrates, while the oxidizing substance may be an oxide of the type  $\text{XO}_3$  or a potassium or sodium salt of the type  $\text{Na}_2(\text{K}_2)\text{XO}_4$ ,

where X is an element selected in the group VIa (chromium, molybdenum and tungsten), or a potassium or sodium bichromate salt (e.g.,  $\text{Na}_2(\text{K}_2)\text{Cr}_2\text{O}_7$ ). The composition of this bath must be such so that its melting temperature is lower than the melting temperature of the zinc.

A current of selected magnitude is passed through the electrolytic cell with the object to be oxidized being used as the anode. The current density may be between 0 to 20  $\text{A}/\text{dm}^2$  and the immersion time may be between 30 sec. and 30 min. In these conditions the voltage across the cell does not exceed ten volts.

Grown on the so processed objects is a layer of complex oxides having characteristics depending on the processing parameters. The object is then extracted, cooled and washed with water.

When the percentage by weight of the oxidizing substance is lower than about 2 percent, the processing is insufficient inasmuch as the zinc dissolves without forming surface oxide layers.

When the percentages of the oxidizing substance varies from 2 percent about to about 10 percent and the current density is less than  $2 \text{ A}/\text{dm}^2$ , the oxides attained are iridescent, conductive and very thin, having a thickness less than 1 micron.

Conversely, solid (thickness up to 10  $\mu$ ), strongly colored, insulating oxides, are attained by baths containing from about 2 to 10 percent of the oxidizing agent and operating with current densities higher than about  $2 \text{ A}/\text{dm}^2$ .

The oxides attained by the method of the invention are made of two well defined layers; an external layer which is variously colored according to the processing undergone and less compact and an internal layer which is light colored, compact and well anchored to the zinc substrate. It is thought that this second layer is probably responsible for the good abrasion resistance found.

For percentages by weight of oxidizing substances higher than 10 percent the current flow produces a quick dissolution of the zinc.

The consistency and the properties of these two layers are determined by the time of oxidation (which may vary from 30 sec. to 30 min. as stated above) and the temperature of oxidation (which may vary between about  $220^\circ\text{C}$  and  $280^\circ\text{C}$ ). By extending the time of oxidation the thickness of the two layers is increased proportionally when the temperature is increased, the external layer takes up varying colorations, while the internal layer substantially increases in uniformity and compactness.

When the sodium chromate  $\text{Na}_2\text{CrO}_4$  or the potassium chromate  $\text{K}_2\text{CrO}_4$  are used as oxidizing agents, due to their lower solubility, their concentration in the bath cannot exceed about 8 percent.

Furthermore, due to their lower oxidizing power, these oxidizing agents are to be present with concentration not lower than 4 percent.

If the oxidizing agent is constituted by sodium bichromate  $\text{Na}_2\text{Cr}_2\text{O}_7$  or potassium bichromate  $\text{K}_2\text{Cr}_2\text{O}_7$ , which have a good solubility, the process can be operated with a concentration of these salts higher than 10 percent. However, also for them the treatment duration has to be not shorter than 1 min.

A variant of the invention consists in executing the surface processing of the zinc by the passivation process, without the use of electrical current, in a bath

made of a mixture of melted salts. The object to be passivated is suitably degreased and immersed in a bath which is substantially the same as the one used as an electrolyte for the anodic oxidation, but with the hexavalent oxide  $\text{CrO}_3$  used as oxidizing substance in a percentage equal or higher than the 10 percent. Formed on the so processed zinc is an oxide protection layer which is similar to the ones attained through the anodic oxidation processing by currents greater than  $2 \text{ A/dm}^2$  and percentages of additive mixture comprised between the 2 and the 10 percent.

A good surface oxidation processing of the zinc in a melted nitrate mixture resulting in the production of a thick and compact oxide layer can thus be attained in either a pure by chemical or an electrolytic manner by suitably selecting the conditions of the processing, and in particular, the bath composition. The oxide protection layers attained by the two methods are not perfectly equivalent however. Oxide layers attained by anodic oxidation and layers attained by passivation are both endowed with a good corrosion resistance, but only the first ones have greatly improved mechanical properties such as resistance to abrasion.

For the tests of the method according to the invention which are here described by way of example, baths of sodium and potassium nitrate equi-molecular mixtures melting at a temperature from  $218^\circ\text{C}$  to  $222^\circ\text{C}$  were prepared, to which chromic anhydride  $\text{CrO}_3$  having a melting point of  $196^\circ\text{C}$  is added in varying percentages.

A cylindric container of inox steel 18/8 having a capacity of 2.5 l was used as electrolysis cell. The temperature was checked by a chromel-alumel thermocouple immersed in the bath. The anodic oxidation process used as cathode the electrolysis cell itself and as anode thin plates of zinc plated steel, the thickness of the zinc layer being  $20\mu$ .

The percentage of  $\text{CrO}_3$  was varied from 0 to 10 percent, the current density from 0 to  $20 \text{ A/dm}^2$  and the bath temperature from  $218^\circ\text{C}$  to  $250^\circ\text{C}$ .

For comparison purposes and for displaying the advantages and some characteristics of the present invention, some tests have been carried out in order to compare the behaviour of thin steel plates coated with a  $20\mu$  zinc layer which have undergone a traditional processing with the behaviour of similar thin plates processed according to the invention.

The traditional processing consists in suitably degreasing and immersing the thin plate into an 1.2 percent aqueous solution of macro-brite L-10-B (chrome passivation and conversion bath of the Ital-Finish, Milan) at the temperature of  $30^\circ\text{C}$ . After 30 sec. immersion the thin plate is extracted from the bath, washed with cold flowing water and subsequently dried in a flow of warm air.

For the corrosion tests the oxidized thin plates were inserted into a saline fog chamber ( $\text{NaCl}$  at 5 percent) at the temperature of  $35^\circ\text{C} \pm 1^\circ\text{C}$ , and their appearance was observed daily. In the course of the test, lasting 1000 hours totally, various corrosion statuses were displayed: (1) decoloration; (2) white oxidation (etching of the zinc coating); (3) red oxidation (etching of the steel substrate).

The results of this test are displayed in the drawing, wherein there is shown the duration and the sequence of the varying corrosion stages for four thin steel plates plated with a  $20\mu$  thick layer of zinc, which are pro-

cessed and exposed in different ways to the corrosion environment.

In the drawing it may be observed as the corrosion resistance properties of a thin plate processed in the traditional manner (example 1) does not differ substantially from those of a thin plate which has undergone an anodic oxidation but by a current density lower than  $2 \text{ A/dm}^2$  and by a  $\text{CrO}_3$ , percentage comprised between 2 and 10 percent (example 2). A substantial improvement of such properties is attained however when the electrolytic current density is greater than  $2 \text{ A/dm}^2$  (example 3). As is illustrated in example 4, the corrosion resistance of the zinc oxidation obtained by passivation is further improved, provided that the concentration of  $\text{CrO}_3$  is equal to or greater than 10 percent.

Responsible for the excellent corrosion resistance of the zinc processed by anodic oxidation or by passivation are the protection layers of thick and compact oxidation formed thereon. Layers having such characteristics are thought to be produced by the high oxidizing conditions resulting from the anodic current or to the high  $\text{CrO}_3$  concentration.

Conversely, the abrasion tests were executed by the Standard Abrasion Tester, Model 503, of the Taber Instruments (North Tonawand, USA) using grinding wheel CS/10 with a load of 500 grs. The abrasion resistance is expressed by the number of revolutions required for conferring an appreciable conductivity on the plate area undergoing the abrasion.

The following table displays the results of tests carried out on thin plates processed according to the method of the invention as previously described for increasing values of the additive percentage ( $\text{CrO}_3$ ) in the electrolytic bath. The table illustrates that as the processing according to the invention generally confers increased resistance, whereas the abrasion resistance of zinc oxidized by the conventional method (example 1) is not increased. In particular, it may be observed that the abrasion resistance is improved, the other conditions being equal, by increasing the bath temperature or the processing duration. Furthermore, example 9 shows that on the contrary the zinc oxidation achieved through passivation is substantially inefficient for improving the abrasion resistance.

Further tests have been carried out by using chromate and bichromate salts as oxidizing agents. Also for these tests a thin steel plate plated with a  $20\mu$  layer of zinc has been immersed in an electrolytic cell.

Example a) the electrolytic bath is made of a solution at 8 percent of potassium chromate  $\text{K}_2\text{CrO}_4$  in an equimolecular mixture of sodium nitrate  $\text{NaNO}_3$  and potassium nitrate  $\text{KNO}_3$  and kept at a temperature of  $230^\circ\text{C}$ . By driving a current of  $1.5 \text{ A/dm}^2$  through the cell for 20 min. a uniform dark green oxide layer is produced on the zinc layer of the steel plate.

Example b) the electrolytic bath is made of a solution at 10 percent of potassium bichromate  $\text{K}_2\text{Cr}_2\text{O}_7$  in an equimolecular mixture of sodium nitrate  $\text{NaNO}_3$  and potassium nitrate  $\text{KNO}_3$  and is maintained at a temperature of  $230^\circ\text{C}$ . By keeping the zinc plated steel plate in the cell for 10 min. and driving through the cell a current of  $2.5 \text{ A/dm}^2$ , on the zinc layer an oxide layer is produced which is dark colored, compact and smooth.

| Example No. | % of CrO <sub>3</sub> in the bath | Current density A/dm <sup>2</sup> | Processing temperature °C | Processing duration | No. of resistance cycle on the abrasion tester |
|-------------|-----------------------------------|-----------------------------------|---------------------------|---------------------|------------------------------------------------|
| 1           | —                                 | —                                 | 30°                       | 20''                | —                                              |
| 2           | 5.5                               | 4                                 | 218°-220°                 | 10'                 | 400-600                                        |
| 3           | 5.5                               | 4                                 | 248°-250°                 | 10'                 | 1000-1200                                      |
| 4           | 8.5                               | 4                                 | 218°-220°                 | 10'                 | 400-500                                        |
| 5           | 8.5                               | 4                                 | 248°-250°                 | 10'                 | 1100-1400                                      |
| 6           | 8.5                               | 4                                 | 218°-220°                 | 5'                  | 200-300                                        |
| 7           | 8.5                               | 8                                 | 218°-220°                 | 5'                  | 500-600                                        |
| 8           | 8.5                               | 8                                 | 218°-220°                 | 10'                 | 300-400                                        |
| 9           | 10                                | 0                                 | 228°-230°                 | 10'                 | 50                                             |

What is claimed is:

1. A method of forming an oxide layer on an object having a surface of zinc comprising the steps of:

a. immersing said object in an electrolytic bath including a solution of hexavalent oxide of the type XO<sub>3</sub>, where X is an element selected from the group consisting of chromium molybdenum and tungsten, in a mixture of melted alkali metal salts, said bath having a melting point lower than the melting point of zinc;

b. passing a direct current of constant density through said bath using said object as an anode.

2. The method of claim 1, wherein said hexavalent oxide is CrO<sub>3</sub> having a percentage in the solution between about 2 and the 10 percent, the current density is at least about 2 A/dm<sup>2</sup> and the process duration is comprised between 30 sec. and 30 min.

3. The method of claim 2, wherein said mixture of alkali metal salts include sodium nitrate and potassium nitrate in an equi-molecular mixture, said bath having an operation temperature between 220°C and 280°C.

4. A method of forming a layer of oxide on an object having a zinc surface comprising the steps of:

a. immersing said object in an electrolytic bath comprising a solution of an acid salt of the type Y<sub>2</sub>XO<sub>4</sub>, where Y is an element selected from the group consisting of sodium and potassium, and X is an element selected from the group consisting of chromium, molybdenum and tungsten, in a melted alkali metal nitrate mixture, the melting temperature of said bath being lower than the melting point of zinc; and

b. passing a direct current of constant density through said bath using said object as an anode.

15 5. The method of claim 4, wherein said salt is K<sub>2</sub>CrO<sub>4</sub> having a percentage in the solution between about 4 and 8 percent, the current density is at least about 2 A/dm<sup>2</sup> and the process duration is comprised between 1 min. and 30 min.

20 6. The method of claim 5, wherein said mixture of alkali metal salts includes sodium nitrate and potassium nitrate in an equi-molecular mixture, said bath having an operation temperature between 220°C and 280°C.

7. A method of forming a layer of oxide on an object having a zinc surface comprising the steps of:

a. immersing said object in a bath comprising a solution of a bichromate salt of the type Y<sub>2</sub>Cr<sub>2</sub>O<sub>7</sub>, where Y is an alkali metal selected from the group consisting of sodium and potassium, in a mixture of melted alkali metal nitrates, the melting temperature of said bath being lower than the melting temperature of zinc; and

b. passing a direct current of constant density through said bath using said object as an anode.

30 8. The method of claim 7, wherein said bichromate salt is K<sub>2</sub>Cr<sub>2</sub>O<sub>7</sub> having in the bath a percentage of at least 2 percent, the current density is at least about 2 A/dm<sup>2</sup> and the process duration is comprised between 1 min. and 30 min.

35 9. The method of claim 8 wherein said mixture of alkali metal salts includes sodium nitrate and potassium nitrate in an equi-molecular mixture, said bath having an operation temperature between 220° and 280°C.

10. The method of claim 1, wherein the alkali metal nitrates in the electrolytic bath include alkaline earth metal nitrates.

\* \* \* \* \*

UNITED STATES PATENT OFFICE  
CERTIFICATE OF CORRECTION

Patent No. 3,852,172

Dated December 3, 1974

Inventor(s) Nicolo Guglielmi and Gianfranco Rolando

It is certified that error appears in the above-identified patent  
and that said Letters Patent are hereby corrected as shown below:

On the first page: Patentees should read --Guglielmi et al. --;  
after "Inventors:" it should read --Nicolo Guglielmi, Settimo Vittone  
and Gianfranco Rolando, Turin, both of Italy--; in "Foreign Application  
Priority Data" delete "June 9, 1971" and substitute --June 11, 1971--.

Signed and sealed this 21st day of January 1975.

(SEAL)

Attest:

McCOY M. GIBSON JR.  
Attesting Officer

C. MARSHALL DANN  
Commissioner of Patents